



US009413075B2

(12) **United States Patent**  
**Avouris et al.**

(10) **Patent No.:** **US 9,413,075 B2**  
(45) **Date of Patent:** **Aug. 9, 2016**

(54) **GRAPHENE BASED STRUCTURES AND METHODS FOR BROADBAND ELECTROMAGNETIC RADIATION ABSORPTION AT THE MICROWAVE AND TERAHERTZ FREQUENCIES**

(75) Inventors: **Phaedon Avouris**, Yorktown Heights, NY (US); **Alberto V. Garcia**, Hartsdale, NY (US); **Chun-Yung Sung**, Poughkeepsie, NY (US); **Fengnian Xia**, Plainsboro, NJ (US); **Hugen Yan**, Ossining, NY (US)

(73) Assignee: **GLOBALFOUNDRIES INC.**, Grand Cayman (KY)

(\*) Notice: Subject to any disclaimer, the term of this patent is extended or adjusted under 35 U.S.C. 154(b) by 705 days.

(21) Appl. No.: **13/523,182**

(22) Filed: **Jun. 14, 2012**

(65) **Prior Publication Data**

US 2013/0335255 A1 Dec. 19, 2013

(51) **Int. Cl.**

**H01Q 17/00** (2006.01)

(52) **U.S. Cl.**

CPC ..... **H01Q 17/00** (2013.01)

(58) **Field of Classification Search**

CPC .... H01Q 17/00; H01Q 17/002; H01Q 17/005  
USPC ..... 342/1-4, 13  
See application file for complete search history.

(56) **References Cited**

U.S. PATENT DOCUMENTS

6,869,581 B2 3/2005 Kishi et al.  
7,015,142 B2 3/2006 DeHeer et al.

|           |      |         |                           |
|-----------|------|---------|---------------------------|
| 7,071,258 | B1   | 7/2006  | Jang et al.               |
| 8,268,180 | B2   | 9/2012  | Arnold et al.             |
| 8,414,964 | B2 * | 4/2013  | Ota et al. .... 427/122   |
| 8,610,617 | B1 * | 12/2013 | Avouris et al. .... 342/3 |
| 9,070,981 | B2 * | 6/2015  | Park ..... B32B 38/08     |
| 9,108,388 | B2 * | 8/2015  | Egami ..... B32B 5/08     |
| 9,210,835 | B2 * | 12/2015 | Avouris ..... B32B 9/04   |
| 9,276,324 | B2 * | 3/2016  | Kelsey ..... B32B 5/02    |

(Continued)

FOREIGN PATENT DOCUMENTS

|    |             |        |
|----|-------------|--------|
| CN | 101010137 A | 8/2007 |
| CN | 101781459 A | 7/2010 |

(Continued)

OTHER PUBLICATIONS

Choi, H., et al "Broadband Electromagnetic Response and Ultrafast Dynamics of Few-Layer Epitaxial Graphene", "Applied Physics Letters", vol. 94 (172102); Mar. 1, 2009, pp. 172102-1 through 172102-3.

(Continued)

*Primary Examiner* — John B Sotomayor

(74) *Attorney, Agent, or Firm* — Anthony Canale; Andrew M. Calderon; Roberts Mlotkowski Safran Cole & Calderon P.C.

(57) **ABSTRACT**

Structures and methods for cloaking an object to electromagnetic radiation at the microwave and terahertz frequencies include disposing a plurality of graphene sheets about the object. Intermediate layers of a transparent dielectric material can be disposed between graphene sheets to optimize the performance. In other embodiments, the graphene can be formulated into a paint formulation or a fabric and applied to the object. The structures and methods absorb at least a portion of the electromagnetic radiation at the microwave and terabyte frequencies.

**6 Claims, 2 Drawing Sheets**



(56)

## References Cited

## U.S. PATENT DOCUMENTS

- 9,306,290 B1 \* 4/2016 Grop ..... H01Q 17/00  
 2007/0284557 A1 \* 12/2007 Gruner et al. ..... 252/500  
 2008/0023396 A1 \* 1/2008 Fugetsu ..... 210/502.1  
 2009/0011204 A1 \* 1/2009 Wang et al. ..... 428/215  
 2009/0017211 A1 \* 1/2009 Gruner et al. ..... 427/258  
 2009/0059474 A1 \* 3/2009 Zhamu et al. ..... 361/503  
 2009/0114890 A1 \* 5/2009 Imholt ..... 252/587  
 2009/0135042 A1 \* 5/2009 Umishita et al. ..... 342/1  
 2009/0146111 A1 \* 6/2009 Shin et al. ..... 252/510  
 2009/0155578 A1 \* 6/2009 Zhamu et al. ..... 428/336  
 2009/0174435 A1 \* 7/2009 Stan et al. ..... 326/112  
 2009/0305135 A1 12/2009 Shi et al.  
 2010/0028681 A1 2/2010 Dai et al.  
 2010/0096181 A1 \* 4/2010 Nakamura et al. ..... 174/394  
 2010/0147188 A1 6/2010 Mamak et al.  
 2010/0149018 A1 6/2010 Umishita et al.  
 2010/0215945 A1 \* 8/2010 Ota et al. ..... 428/323  
 2010/0279426 A1 \* 11/2010 Tour et al. ..... 436/149  
 2011/0089404 A1 4/2011 Marcus et al.  
 2011/0108805 A1 5/2011 Okai  
 2011/0108806 A1 \* 5/2011 Davidovic et al. ..... 257/29  
 2011/0163298 A1 7/2011 Sung  
 2011/0175060 A1 7/2011 Okai  
 2011/0186818 A1 \* 8/2011 Bowers et al. ..... 257/29  
 2011/0210282 A1 9/2011 Foley  
 2011/0210314 A1 9/2011 Chung et al.  
 2011/0240946 A1 10/2011 Miao  
 2011/0250427 A1 10/2011 Kotov et al.  
 2011/0278545 A1 11/2011 Voutilainen et al.  
 2011/0300338 A1 \* 12/2011 Shin et al. ..... 428/156  
 2011/0303121 A1 12/2011 Geim et al.  
 2011/0303899 A1 12/2011 Padhi et al.  
 2011/0320142 A1 \* 12/2011 Surman et al. ..... 702/50  
 2012/0001761 A1 \* 1/2012 Voutilainen et al. ..... 340/600  
 2012/0007913 A1 1/2012 Jang  
 2012/0039344 A1 2/2012 Kian et al.  
 2012/0058350 A1 \* 3/2012 Long et al. ..... 428/446  
 2012/0064409 A1 \* 3/2012 Zhamu et al. ..... 429/221  
 2012/0068160 A1 \* 3/2012 Yamazaki et al. ..... 257/29  
 2012/0080086 A1 4/2012 Yoon et al.  
 2012/0170354 A1 \* 7/2012 Voutilainen et al. ..... 365/149  
 2012/0213994 A1 8/2012 Jafry et al.  
 2012/0265122 A1 10/2012 El-Shall et al.  
 2012/0288433 A1 \* 11/2012 Sutter et al. ..... 423/445 B  
 2012/0308884 A1 12/2012 Oguni et al.  
 2012/0325296 A1 12/2012 Woo et al.  
 2013/0001515 A1 1/2013 Li et al.  
 2013/0048952 A1 2/2013 Chen et al.  
 2013/0068521 A1 3/2013 Hong et al.  
 2013/0113081 A1 \* 5/2013 Chen et al. ..... 257/602  
 2013/0333937 A1 12/2013 Avouris et al.  
 2013/0335254 A1 \* 12/2013 Avouris et al. ..... 342/3  
 2013/0335255 A1 \* 12/2013 Avouris ..... H01Q 17/00  
 342/4  
 2014/0004344 A1 \* 1/2014 Kim et al. ..... 428/367  
 2014/0011027 A1 \* 1/2014 Kim et al. ..... 428/367

## FOREIGN PATENT DOCUMENTS

- CN 102502611 A1 6/2012  
 DE 102013210161 A1 \* 12/2013 ..... H01Q 17/002  
 EP 2409951 A1 \* 1/2012  
 ES 2369953 A1 12/2011

- JP 2012025652 A \* 2/2012  
 WO 2008056123 A1 5/2008  
 WO WO2010022353 A1 2/2010  
 WO 2011108878 A2 9/2011  
 WO 2012094498 A2 7/2012

## OTHER PUBLICATIONS

- Fugetsu, Bunshi. et al. "Graphene Oxide as Dyestuffs for the Creation of Electrically Conductive Fabrics", "Carbon", vol. 48 (12); Oct. 2010, pp. 1-27.  
 Hesjedal, Thorsten. et al. "Continuous Roll-to-Roll Growth of Graphene Films by Chemical Vapor Deposition", "Applied Physics Letters", vol. 98 (133106); Feb. 8, 2011, pp. 133106-1 through 133106-3.  
 Lee, Chul. et al. "Optical Response of Large Scale Single Layer Graphene", "Applied Physics Letters", vol. 98 (071905); Aug. 26, 2011, pp. 071905-1 through 071905-3.  
 Liu, Jianwei. et al. "Doped Graphene Nanohole Arrays for Flexible Transparent Conductors", "Applied Physics Letters", vol. 99 (023111); Mar. 31, 2011, pp. 023111-1 through 023111-3.  
 Ludwig, Alon. et al. "ODark Materials Based on Graphene Sheet Stacks", "Optics Letters", vol. 36, No. 2; Jan. 15, 2011, pp. 106-107.  
 LV, Ruitao. et al. "Carbon Nanotubes Filled with Ferromagnetic Alloy Nanowires: Lightweight and Wide-Band Microwave Absorber", "Applied Physics Letters", vol. 93 (223105); Jul. 19, 2008, pp. 223105-1 through 223105-3.  
 Zhang, X.F., et al. "Microwave Absorption Properties of the Carbon-Coated Nickel Nanocapsules", "Applied Physics Letters", vol. 89 (053115); May 9, 2006, pp. 053115-1 through 053115-2.  
 Lv et al; Towards new graphene materials: Doped graphene sheets and nanoribbons, Materials Letters, 78 (2012), 209-218.  
 Yan, et al; Infrared Spectroscopy of Tunable Dirac Terahertz Magneto-Plasmons in Graphene, Nano Lett. 2012, 12, 3766-3771.  
 Yan, et al; Tunable infrared plasmonic devices suing graphene/insulator stacks. Nature Nanotechnology. vol. 7, May 2012-330.  
 De Bellis, G. et al.; "Electromagnetic Absorbing Nanocomposites including Carbon Fibers, Nanotubes and Graphene Nanoplatelets," Electromagnetic Compatibility (EMC), 2010 IEEE International Symposium, vol., No., pp. 202-207, Jul. 25-30, 2010.  
 Sekine, T., et al.; "Transparent and Double-Sided Wave Absorber with Specified Reflection and Transmission Coefficients," Electromagnetic Compatibility—EMC Europe, 2009 International Symposium, vol., No., pp. 1-3, Jun. 11-12, 2009.  
 Tennant, A.; Chambers, B.; "Phase switched radar absorbers," Antennas and Propagation Society International Symposium, 2001. IEEE , vol. 4, No., pp. 340-343 vol. 4, 2001.  
 Yu, H., et al.; (Abstract), Graphene/Polyaniline Nanorod Arrays: Synthesis and Excellent Electromagnetic absorption properties. Journal of Materials Chemistry, 2012; 22(40), 21679-21685.  
 Office Action issued in German Application No. 10 2013210162.7, dated Jul. 7, 2015; 6 pages.  
 LV, Ruitao. et al. "Towards new graphene materials: Doped graphene sheets and nanoribbons", Materials Letters, vol. 93 (2012); pp. 209-218.  
 Office Action issued in German Application No. 10 2013210161.9, dated Oct. 16, 2015; 8 pages.  
 Response to Office Action Filed in German Application No. 102013210161.9, dated Dec. 10, 2015; 13 pages including clean and marked up claims.

\* cited by examiner



FIG. 1



FIG. 2



FIG. 3



FIG. 4

## 1

**GRAPHENE BASED STRUCTURES AND  
METHODS FOR BROADBAND  
ELECTROMAGNETIC RADIATION  
ABSORPTION AT THE MICROWAVE AND  
TERAHERTZ FREQUENCIES**

**BACKGROUND**

The present disclosure generally relates to structures and methods for absorbing broadband electromagnetic waves using graphene, and more particularly, to methods and structures of graphene sheets configured to absorb the broadband electromagnetic waves at the microwave and terahertz frequencies being emitted from an electromagnetic wave generating source.

The development of broadband absorption materials at the microwave and terahertz spectrum range is currently being investigated for numerous commercial and military applications. For example, terahertz radar systems are capable of probing the detailed structure of targets on a sub-millimeter scale while being able to distinguish between materials in terms of the spectral dependence of absorption. For military applications, weapons or personnel could be detected through catalogue or thin foliage and targets discriminated from background on the basis of spectral response. The use of broadband absorption materials that completely absorb the incident electromagnetic waves of interest, e.g., the terahertz frequencies, such that no transmission and reflection occurs can be used to effectively hide the target. However, most known material systems for such purposes rely on resonance peaks in the absorption spectrum and as such, a broadband solution is still lacking.

**SUMMARY**

According to an embodiment, a structure for absorbing electromagnetic radiation in the microwave and terahertz frequencies comprises a plurality of graphene sheets on or about the object to be cloaked from the electromagnetic radiation. In some instances, the cloaking structure may further comprise a transparent dielectric layer intermediate adjacent graphene sheets.

In another embodiment, a structure for absorbing broadband electromagnetic radiation in the microwave and terahertz frequencies comprises a plurality of graphene sheets configured on or about an object so as to absorb broadband electromagnetic radiation in the microwave and terahertz frequencies.

In another embodiment, a removable structure for absorbing electromagnetic radiation in the microwave and terahertz frequencies comprises a fabric comprising graphene, wherein the fabric is configured to removably wrap about an object, wherein the graphene is in an amount effective to absorb at least a portion of the electromagnetic radiation at the microwave and/or terahertz frequencies.

Additional features and advantages are realized through the techniques of the present invention. Other embodiments and aspects of the invention are described in detail herein and are considered a part of the claimed invention. For a better understanding of the invention with advantages and features, refer to the description and to the drawings.

**BRIEF DESCRIPTION OF THE SEVERAL  
VIEWS OF THE DRAWINGS**

The subject matter which is regarded as the invention is particularly pointed out and distinctly claimed in the claims at

## 2

the conclusion of the specification. The forgoing and other features, and advantages of the invention are apparent from the following detailed description taken in conjunction with the accompanying drawings in which:

5 FIG. 1 illustrates transmission spectrum of a single layer of graphene in the far infrared and terahertz regions.

FIG. 2 illustrates an electromagnetic broadband absorption structure for absorbing electromagnetic radiation at the microwave and terahertz spectrums, the structure including a 10 plurality of graphene sheets according to an embodiment.

FIG. 3 illustrates an electromagnetic broadband absorption structure for absorbing electromagnetic radiation at the microwave and terahertz spectrums, the structure including a 15 plurality of graphene sheets separated by transparent intermediate layers according to an embodiment.

FIG. 4 illustrates an electromagnetic broadband absorption structure for absorbing electromagnetic radiation at the microwave and terahertz spectrums, the structure including a 20 coating containing graphene flakes according to an embodiment.

**DETAILED DESCRIPTION**

Disclosed herein are electromagnetic broadband absorption structures and methods for absorbing at least a portion of the electromagnetic radiation emitted from an electromagnetic radiation source at the microwave and terahertz frequencies. By providing broadband absorption of electromagnetic waves at the microwave and terahertz frequencies, an object 25 can effectively be hidden at these frequencies since the broadband electromagnetic waves are absorbed and no transmission or reflection occurs. As used herein, the term "microwave" generally refers to the wavelength range of 1 millimeter to 1 meter (i.e., 300 MHz to 300 GHz) whereas the 30 term "terahertz" generally refers sub-millimeter wave energy that fills the wavelength range between 1000 to 100 microns (i.e., 300 GHz to 3 THz)

The electromagnetic broadband absorption structures are 35 generally formed from a plurality of graphene sheets, wherein 40 the electromagnetic broadband absorption structure is effective to absorb at least a portion of the electromagnetic radiation at the microwave and terahertz frequencies. The number of graphene sheets will generally depend on the intended 45 application and the desired minimal reflection for the particular application. A typical graphene "layer" may comprise a single sheet or multiple sheets of graphene, for example, between 1 sheet and 1000 sheets in some embodiments, and between about 10 sheets and 100 sheets in other embodiments. In most embodiments, the resulting graphene layer 50 comprised of the graphene sheets can have a thickness of about 1 nanometer to about 100 nanometers, and a thickness of about 10 nm to about 80 nm in other embodiments.

Graphene is a two dimensional allotrope of carbon atoms 55 arranged in a planar, hexagonal structure. It features useful electronic properties including bipolarity, high purity, high mobility, and high critical current density. Electron mobility values as high as 200,000 cm<sup>2</sup>/Vs at room temperature have been reported.

Structurally, graphene has hybrid orbitals formed by sp<sup>2</sup> 60 hybridization. In the sp<sup>2</sup> hybridization, the 2s orbital and two of the three 2p orbitals mix to form three sp<sup>2</sup> orbitals. The one remaining p-orbital forms a pi-bond between the carbon atoms. Similar to the structure of benzene, the structure of graphene has a conjugated ring of the p-orbitals which exhibits 65 its a stabilization that is stronger than would be expected by the stabilization of conjugation alone, i.e., the graphene structure is aromatic. Unlike other allotropes of carbon such as

diamond, amorphous carbon, carbon nanofoam, or fullerenes, graphene is not an allotrope of carbon since the thickness of graphene is one atomic carbon layer i.e., a sheet of graphene does not form a three dimensional crystal.

Graphene has an unusual band structure in which conical electron and hole pockets meet only at the K-points of the Brillouin zone in momentum space. The energy of the charge carriers, i.e., electrons or holes, has a linear dependence on the momentum of the carriers. As a consequence, the carriers behave as relativistic Dirac-Fermions having an effective mass of zero and moving at the effective speed of light of  $c/10^6$  m/sec. Their relativistic quantum mechanical behavior is governed by Dirac's equation. As a consequence, graphene sheets have a large carrier mobility of up to 60,000 cm<sup>2</sup>/V-sec at 4K at 300K, the carrier mobility is about 15,000 cm<sup>2</sup>/V-sec. Also, quantum Hall effect has been observed in graphene sheets.

The linear dispersion of graphene around the K (K') point leads to constant interband absorption (from valence to conduction bands, about 2.3%) of vertical incidence light in a very broadband wavelength range. More interestingly, at the microwave and terahertz frequency ranges, intraband absorption dominates and a single layer can absorb as much as 30% at a light wavelength of 300 microns depending on the carrier concentration in the graphene as evidenced by the transmission spectrum provided in FIG. 1. As a result, utilization of graphene for microwave and terahertz frequency absorption has numerous advantages such as being an ultra-thin and efficient absorption layer relative to other materials. Moreover, because graphene is a one atom thick monolayer sheet formed of carbon atoms packed in a honeycomb crystalline lattice, wherein each carbon atom is bonded to three adjacent carbon atoms via sp<sup>2</sup> bonding, the overall thickness required to provide effective absorption is minimal is on the order of a few nanometers. As such, the use of graphene sheets provides minimal added weight to the object to be shielded, has broadband absorption capabilities, and provides greater versatility than prior art structures. Moreover, graphene is generally recognized for its high mechanical strength and high stability which are desirable properties for most applications.

The graphene sheets can be made by any suitable process known in the art including mechanical exfoliation of bulk graphite, for example, chemical deposition, growth, or the like. Currently, among the conventional methods of forming a graphene layer, the method of forming the graphene layer by chemical vapor deposition is being frequently used because a large area graphene layer can be produced at a relatively low cost.

By way of example only, chemical vapor deposition (CVD) onto a metal (i.e., foil) substrate can be used to form the graphene sheets. To form the graphene layer by chemical vapor deposition, a precursor is selected so that the catalytic decomposition of the precursor forms the graphene layer. The precursor may be a gas, liquid, or solid hydrocarbon such as methane, ethylene, benzene, toluene, and the like. The precursor may also include and be mixed with other materials such as hydrogen gas, for example.

The CVD process may be implemented at atmospheric pressure or the vacuum chamber of the CVD apparatus may be evacuated below atmospheric pressure. In one embodiment, the vacuum chamber is pressurized between 100 mTorr and 500 m Torr. The CVD apparatus may also be configured to heat the substrate to be coated with the graphene. For example, the substrate can be heated up to about 1200° C. or higher as may be desired with some precursors and applications.

Chemical exfoliation may also be used to form the graphene sheets. These techniques are known to those of skill in the art and thus are not described further herein.

The graphene can be formed on a substrate as may be desired in some applications. The particular substrate is not intended to be limited and may even include the electromagnetic radiation source itself. For example, the structural material may include foams, honeycombs, glass fiber laminates, Kevlar fiber composites, polymeric materials, or combinations thereof. Non-limiting examples of suitable structural materials include polyurethanes, silicones, fluorosilicones, polycarbonates, ethylene vinyl acetates, acrylonitrile-butadiene-styrenes, polysulfones, acrylics, polyvinyl chlorides, polyphenylene ethers, polystyrenes, polyamides, nylons, polyolefins, poly(ether ether ketones), polyimides, polyetherimides, polybutylene terephthalates, polyethylene terephthalates, fluoropolymers, polyesters, acetals, liquid crystal polymers, polymethylacrylates, polyphenylene oxides, polystyrenes, epoxies, phenolics, chlorosulfonates, polybutadienes, neoprenes, nitriles, polyisoprenes, natural rubbers, and copolymer rubbers such as styrene-isoprene-styrenes, styrene-butadiene-styrenes, ethylene-propylenes, ethylene-propylene-diene monomers (EPDM), nitrile-butadienes, and styrene-butadienes (SBR), and copolymers and blends thereof. Any of the forgoing materials may be used unfoamed or, if required by the application, blown or otherwise chemically or physically processed into open or closed cell foam.

The shape of the substrate is not intended to be limited. For example, the substrate may have planar and/or curvilinear surfaces such as may be found in foils, plates, tubes, and the like.

Once the graphene sheets are formed, the sheets can be deposited onto a desired object using conventional lift-off techniques or may be deposited directly onto the substrate of interest. In general, the sheets are deposited one on top of another to form the film. Thus, by way of example only, the graphene film can comprise a stack of multiple graphene sheets (also called layers). The term "substrate" is used to generally refer to any suitable substrate on which one would want to deposit a graphene film and have that particular substrate effectively hidden from electromagnetic radiation at the microwave and terahertz frequencies.

In one embodiment shown in FIG. 2, the electromagnetic broadband absorption structure 10 for absorbing electromagnetic radiation at the microwave and terahertz frequencies includes a plurality of graphene sheets 14<sup>1</sup>, 14<sup>2</sup>, . . . 14<sup>n</sup> directly transferred to the substrate of interest 12. The number of graphene sheets utilized will generally vary depending on the intended application and the desired level of minimal reflection for the particular application.

In another embodiment shown in FIG. 3, the electromagnetic broadband absorption structure 20 disposed on or about an object 22 for absorbing electromagnetic radiation at the microwave and terahertz frequencies includes one or more graphene sheets 24<sup>1</sup>, 24<sup>2</sup>, . . . 24<sup>n</sup>, wherein intermediate the graphene sheets are transparent intermediate dielectric layer 26.

In one embodiment, suitable dielectric materials include, without limitation, silicon dioxide, silicon nitride, porous silicon dioxide, polyimide, polynorbornenes, benzocyclobutene, methylsilsesquioxanes, a doped glass layer, such as phosphorus silicate glass, boron silicate glass, and the like. In other embodiments, the dielectric layer can be a low k dielectric layer, wherein low k generally refers to materials having a dielectric constant less than silicon dioxide. Exemplary low k dielectric materials include, without limitation, SiLK® from Dow Chemical, Coral® from Novellus, Black Dia-

mond® from Applied Materials, and spin on dielectrics can be used. Coral® can be described generically as a SiCOH dielectric. Depending upon the particular dielectric material, dielectric layer can be formed by chemical vapor deposition deposited (CVD), plasma enhanced chemical vapor deposition (PECVD), atmospheric deposition as well as spin on techniques. In one embodiment, the dielectric layer is a chemical vapor deposited material, such as silicon dioxide or silicon nitride, deposited between adjacent graphene layers. By adjusting the refractive index and thickness of the intermediate dielectric layers, the performance of the structure can be optimized for a particular application.

In another embodiment shown in FIG. 4, the electromagnetic broadband absorption structure 30 for absorbing electromagnetic radiation at the microwave and terahertz frequencies includes one or more coatings 34 of a paint formulation including graphene flakes as a pigment applied to a surface of an object 32 for cloaking. The amount of graphene flakes can generally be varied within the paint formulation. However, a high concentration is generally preferred so as to minimize coating thickness. The other components of the paint formulation including a binder, e.g., latex, can be those conventionally employed in paint formulations so long as the other components do not interfere with the absorption properties provided by the graphene flakes. For example, the binder may include synthetic or natural resins such as alkyds, acrylics, vinyl-acrylics, vinyl acetate/ethylene (VAE), polyurethanes, polyesters, melamine resins, epoxy, or oils. Binders may be categorized according to the mechanisms for drying or curing. Although drying may refer to evaporation of the solvent or thinner, it usually refers to oxidative cross-linking of the binders and is indistinguishable from curing. Some paints form by solvent evaporation only, but most rely on cross-linking processes. The paint formulation can also include a wide variety of miscellaneous additives, which are usually added in small amounts. By way of example, typical additives may be included to modify surface tension, improve flow properties, improve the finished appearance, increase wet edge, improve pigment stability, impart antifreeze properties, control foaming, control skinning, etc. Other types of additives include catalysts, thickeners, stabilizers, emulsifiers, texturizers, adhesion promoters, UV stabilizers, flatteners (de-glossing agents), biocides to fight bacterial growth, and the like.

Once applied to the substrate of interest, the painted coating can provide high absorption at the microwave and terahertz frequencies once applied to the substrate of interest.

Optionally, a fabric or cloth including the graphene flakes can be provided to provide an object to be cloaked with uncloaking capabilities, when desired. Moreover, the fabric or cloth can be shared with multiple objects. The terms fabric or cloth generally refers to a flexible artificial material that is made by a network of natural or artificial fibers. The fabric can be impregnated and/or woven with the graphene flakes, which may include a binder to facilitate adhesion of the graphene flakes to the fabric. The fabric itself is not intended to be limited to any particular type. The graphene flakes may be prepared by mechanical exfoliation as graphite bulk to yield micron sized graphene flakes such as is generally described in US Patent Publication No. 2010/0147188, incorporated herein by reference in its entirety. It may also be commercially obtained from GrafTech INternational Ltd, Parma, Ohio as GRAFGUARD®.

Substrates that include graphene layers and/or graphene flakes as discussed above provide reduced terahertz microwave and infrared crossections. As a result, the substrate itself will be effectively hidden since the graphene layers and/or

graphene flakes are low transmitting and low reflectively materials, the degree of which will generally depend on the thickness and density of the graphene. Such optimization is well within the skill of those of ordinary skill in the art.

5 It will be understood that when an element or layer is referred to as being "on," "interposed," "disposed," or "between" another element or layer, it can be directly on, interposed, disposed, or between the other element or layer or intervening elements or layers may be present.

10 It will be understood that, although the terms first, second, third, and the like may be used herein to describe various elements, components, regions, layers and/or sections, these elements, components, regions, layers and/or sections should not be limited by these terms. These terms are only used to 15 distinguish one element, component, region, layer or section from another element, component, region, layer or section. Thus, first element, component, region, layer or section discussed below could be termed second element, component, region, layer or section without departing from the teachings 20 of the present invention.

The terminology used herein is for the purpose of describing particular embodiments only and is not intended to be limiting of the invention. As used herein, the singular forms "a", "an" and "the" are intended to include the plural forms as well, unless the context clearly indicates otherwise. It will be further understood that the terms "comprises" and/or "comprising," when used in this specification, specify the presence of stated features, integers, steps, operations, elements, and/or components, but do not preclude the presence or addition 30 of one or more other features, integers, steps, operations, elements, components, and/or groups thereof.

The corresponding structures, materials, acts, and equivalents of all means or step plus function elements in the claims below are intended to include any structure, material, or act 35 for performing the function in combination with other claimed elements as specifically claimed. The description of the present invention has been presented for purposes of illustration and description, but is not intended to be exhaustive or limited to the invention in the form disclosed. Many 40 modifications and variations will be apparent to those of ordinary skill in the art without departing from the scope and spirit of the invention. The embodiment was chosen and described in order to best explain the principles of the invention and the practical application, and to enable others of ordinary skill in the art to understand the invention for various 45 embodiments with various modifications as are suited to the particular use contemplated.

What is claimed is:

- 50 1. A cloaking structure for absorbing broadband electromagnetic radiation in the microwave and terahertz frequencies, the structure consisting of:  
a plurality of graphene sheets deposited on an object so as to absorb broadband electromagnetic radiation in the microwave and terahertz frequencies; and  
a transparent dielectric layer intermediate adjacent graphene sheets, wherein the cloaking structure is configured about the object, wherein the object is a source of the electromagnetic radiation.
- 55 2. The structure of claim 1, wherein the object has a curvilinear surface.
3. The structure of claim 1, wherein the plurality of graphene sheets have a thickness of about 1 nanometer to about 100 nanometers.
- 60 4. The structure of claim 1, wherein the plurality of graphene sheets have a thickness of about 10 nanometers to about 80 nanometers.

5. The structure of claim 1, wherein the plurality of graphene sheets is between about 10 sheets to about 100 sheets.

6. The structure of claim 1, wherein the transparent dielectric layer comprises any one of silicon dioxide, silicon nitride, porous silicon dioxide, polyimide, polynorbornenes, benzocyclobutene, methylsilsequioxanes, phosphorus silicate glass, or boron silicate glass. 5

\* \* \* \* \*